

## UNITED STATES PATENT OFFICE.

HERBERT KRANICH, OF BROOKLYN, NEW YORK, ASSIGNOR TO S. STERNAU & COMPANY, INC., OF BROOKLYN, NEW YORK, A CORPORATION OF NEW YORK.

## SOLIDIFIED LIQUID FUEL AND PROCESS OF MAKING THE SAME.

No Drawing.

Application filed June 7, 1919. Serial No. 302,564.

*To all whom it may concern:*

Be it known that I, HERBERT KRANICH, a citizen of the United States, and a resident of the borough of Brooklyn, county of Kings, city and State of New York, have invented a certain new and useful Solidified Liquid Fuel and Process of Making the Same, of which the following is a specification.

10 The invention relates to a solid fuel composed mainly of alcohol, and more particularly to such a product as may be made in the container in which it is vended and burned. The fuel may also be made in bulk and formed to any desired configuration or shape, cubical for example, and will retain its shape without being confined in a container of that shape.

15 The objects of the invention are the production of a solid fuel which will be economical of manufacture; which will be infusible and retain its solid form until consumed; which, when consumed, will leave practically no residue; which will be stable and possess good keeping qualities; which will burn with a flame of intense heat and for a longer time than prior solid alcohol fuels; which will not form a crust when the flame is extinguished; which may readily be rekindled; which is non-explosive; and which is, therefore, safe to manufacture, transport and operate.

20 A further object of the invention is to provide a process of producing a solidified fuel composed mainly of alcohol, and having the above mentioned characteristics, which may be expeditiously carried out, and wherein losses by evaporation, and otherwise, may be greatly reduced.

25 These and further objects will more fully appear in the following specification and claims.

30 By means of the invention an infusible, solid fuel composed mainly of alcohol, and having a base of nitro cellulose and cellulose acetate is produced.

35 Broadly stated the invention comprises dissolving cellulose having a nitrogen content which renders it soluble in acetone, and designated herein as pyroxylene, in a mixture of alcohol and a solvent, adding a hygroscopic salt solution, and solidifying the mixture by the introduction of a coagulating liquid.

40 In carrying out what is now considered

the preferred process of the invention I provide an alcohol mixture, preferably of approximately 20% by volume of wood alcohol, and 80% by volume of commercial grain alcohol. It is to be understood that if grain alcohol denatured with wood spirits is used wood alcohol is added to form the mixture desired. To the alcohol mixture is added a dry nitro cellulose (pyroxylene) in the proportions of about 17% by weight pyroxylene to about 83% by weight of the alcohol. The pyroxylene is insoluble in this mixture.

45 To the pyroxylene alcohol mixture is added a small proportion, approximately 1% to 1½%, of a pyroxylene solvent such as commercial acetone, and the mixture goes into solution forming a heavy, viscous mixture. If desired the pyroxylene may be dissolved in the acetone before mixing with the alcohol, but the former method is preferred as the low boiling point of the ketone and its pronounced hygroscopicity make such a solution difficult.

50 I next prepare an approximately 5% solution of ammonium nitrate by dissolving commercial ammonium nitrate in alcohol, preferably the mixture above described, and heating the solution to about 60° C. The water in the alcohol is taken up by the ammonium nitrate and the latter is present in an aqueous solution in the mixture. This hot solution will have a solvent action on the alcohol-pyroxylene-acetone mass, and when the mixture contains about 75% of the solvent, a thin, limpid liquid will be formed. This liquid is placed in a receptacle, which may be the container in which the fuel is to be vended and burned.

55 The limpid liquor in the receptacle is now gelatinized by the admixture of a liquid coagulant. Such a coagulant may be formed by treating a suitably prepared cellulose acetate with diluted alcohol and heating until solution is effected. Such a suitably prepared cellulose acetate may be prepared by mixing cotton, acetic acid, acetic anhydride and a small proportion of sulphuric acid, and allowing the mixture to stand until it is transformed into a thick viscous syrup. Such an ester has been given the trade name of "Sericose". This mass on cooling sets to a firm jell, and must be used before it cools sufficiently to jell. The fluidity of the pyroxylene solution produced

80

85

90

95

100

105

110

by the admixture of the ammonium nitrate solution makes for the quick and thorough dissemination of the liquid coagulant throughout the mass. The sericose in the 5 coagulating solution should be about 1%.

The dissolved sericose is preferably injected into the nitrocellulose-alcohol-ammonium nitrate mass until the sericose forms about 20% of the new mixture, and 10 the total mass in the receptacle sets, on cooling, to a firm coagulum.

The coagulant diffuses into the nitrocellulose solution which is a true colloid and partially precipitates the nitrocellulose from 15 its colloidal solution into an emulsion colloid solution, and the ammonium nitrate in the mixture has the effect of causing the nitrocellulose, in its emulsion or partially precipitated form, to swell, as it were, 20 whereby its capacity for absorbing the alcohol will be increased. As the coagulant diffuses into the mass as a whole the percentage of the solvent of the sericose relatively to the cericose is reduced and the latter 25 gelatinizes on cooling in the alcohol and the entire mass sets to a solid coagulum.

Instead of forming the product in the receptacle in which it is to be vended and burned, the final mixture may be made in 30 bulk and after cooling cut or otherwise formed into cubes, or other shapes, and packed in any desired manner.

The gelatinous sericose tempers the burning rate, reduces the inflammability of the 35 nitrocellulose, and produces a slower burning mixture.

The fuel produced by the process of this application is a dry, solid mass which will retain the liquid combustible under handling; from which the liquid will not exude; which, when ignited will burn slowly without liquefaction and will leave practically no residue.

The product is non-explosive; may be 45 easily ignited either in a container or in the open; will remain perfectly dry while burning; will become cool immediately the flame is extinguished, and may be readily reignited.

It is to be understood that while the mixture of ethyl and methyl alcohol given is 50 preferred, pure alcohol, or ordinary denatured alcohol may be employed, in which case the proportion of pyroxylene solvent will be changed.

Instead of using acetone, any other known solvent of pyroxylene may be employed.

Instead of using a hygroscopic salt, such as ammonium nitrate, to absorb the water 60 of the alcohol, alcohol of higher proof than the ordinary commercial article may be used, and the process may be carried out in the manner and proportions above described for making the limpid solution except that the 65 salt is omitted. The high proof alcohol will

have the same effect on the emulsified nitrocellulose as will the ammonium nitrate. A thin, limpid solution is formed, and the mixture is made cold. The heated coagulant will be added as before and on cooling will 70 solidify the mass. If desired instead of utilizing high proof alcohol, the ordinary commercial article may be dehydrated as by the use of lime or other dehydrant and then used. In such a product the nitro cellulose 75 will not absorb the alcohol as readily as before. When ammonium nitrate is dissolved in commercial alcohol, or when alcohol of higher proof than the commercial article, is employed as the solvent of the alcohol 80 pyroxylene acetone mass, more of the alcohol will be taken up by the mass than if 95% alcohol alone were used. Applicant does not know why this is so, and the explanation given is to the best of his knowledge and 85 belief.

Having now described my invention what I claim and desire to secure by Letters Patent, is:

1. A solid infusible fuel, comprising a solution of approximately 5 parts alcohol, 1 part pyroxylene, 1 part acetone, 75 parts of a 5% solution of ammonium nitrate and dissolved in alcohol, and a small proportion of sericose.

2. A solid infusible fuel, comprising a solution of approximately 4 parts grain alcohol, 1 part wood alcohol, 1 part pyroxylene, 1 part acetone, 75 parts of a 5% solution of ammonium nitrate and dissolved in alcohol, 100 and a small portion of sericose.

3. A solid infusible fuel composed mainly of alcohol, and comprising pyroxylene, acetone, ammonium nitrate, and sericose, substantially as described.

4. A solid, infusible fuel composed mainly of alcohol, and comprising pyroxylene, acetone, ammonium nitrate, a cellulose acetate and water substantially as described.

5. The process of making an infusible solid alcohol fuel, which comprises adding pyroxylene to a mixture of grain and wood alcohols, adding a solvent of pyroxylene to the mixture to produce a heavy viscous solution, adding a diluting liquid to the said 110 solution, and adding a liquefied coagulant to the mass.

6. The process of making an infusible solid alcohol fuel, which comprises mixing pyroxylene with alcohol, adding acetone in a 120 sufficient quantity to produce a heavy viscous solution, adding an alcoholic solution of a hygroscopic salt to the viscous solution, and adding sericose to coagulate the mass.

7. The process of making an infusible solid alcohol fuel, which comprises mixing dry pyroxylene with alcohol, adding commercial acetone to the mixture to dissolve the pyroxylene, adding commercial ammonium nitrate dissolved in commercial alco- 125 130

hol to the solution, and adding sericose dissolved in alcohol to the solution to solidify the mass.

8. The process of making an infusible solid alcohol fuel, which comprises mixing dry pyroxyline with alcohol, adding commercial acetone to the mixture to dissolve the pyroxyline alcohol mixture, adding a heated solution of ammonium nitrate and alcohol to the first mentioned solution, and adding a heated solution of sericose and dilute alcohol to the solution whereby the mass will solidify on cooling.

9. The process of making a solid, infusible alcohol fuel, which comprises dissolving a mixture of pyroxyline and alcohol in an inflammable solvent, and adding a heated solution of sericose to the pyroxyline solution, whereby the cooling of the sericose solution will coagulate the entire mass.

This specification signed and witnessed this sixth day of June, 1919.

HERBERT KRANICH.

Witnesses:

CHARLES C. COLINA,  
A. E. RENTON.